



US007704662B2

(12) **United States Patent**  
**Kmiecik-Lawrynowicz et al.**

(10) **Patent No.:** **US 7,704,662 B2**  
(45) **Date of Patent:** **Apr. 27, 2010**

(54) **SINGLE COMPONENT DEVELOPER**

(75) Inventors: **Grazyna E Kmiecik-Lawrynowicz**, Fairport, NY (US); **Daniel W Asarese**, Honeoye Falls, NY (US); **Maura A Sweeney**, Irondequoit, NY (US); **Robert D Bayley**, Fairport, NY (US)

(73) Assignee: **Xerox Corporation**, Stamford, CT (US)

(\*) Notice: Subject to any disclaimer, the term of this patent is extended or adjusted under 35 U.S.C. 154(b) by 279 days.

(21) Appl. No.: **11/861,695**

(22) Filed: **Sep. 26, 2007**

(65) **Prior Publication Data**

US 2009/0081572 A1 Mar. 26, 2009

(51) **Int. Cl.**

**G03G 9/13** (2006.01)

(52) **U.S. Cl.** ..... **430/109.4**; 430/111.4; 430/137.14

(58) **Field of Classification Search** ..... **430/137.14**  
430/109.4, 111.4

See application file for complete search history.

(56) **References Cited**

**U.S. PATENT DOCUMENTS**

2007/0048643 A1 \* 3/2007 Kmiecik-Lawrynowicz et al. .... 430/108.6  
2007/0190441 A1 \* 8/2007 Sweeney et al. .... 430/108.4

\* cited by examiner

*Primary Examiner*—John L Goodrow

(74) *Attorney, Agent, or Firm*—Carter, DeLuca, Farrell & Schmidt LLP

(57) **ABSTRACT**

A toner for use in a single component development system, said toner including emulsion aggregation toner particles with a styrene acrylate polymer binder resin having a molecular weight Mw of from about 50 to about 100 Kpse and a number average molecular weight (Mn) of from about 10 to about 30 Kpse, a wax selected from the group consisting of polypropylene and polyethylene, and at least one colorant, wherein the toner particles have an onset glass transition temperature of from about 50° C. to about 60° C., and a circularity of from about 0.950 to about 0.990.

**12 Claims, No Drawings**

## 1

## SINGLE COMPONENT DEVELOPER

## CROSS REFERENCE TO RELATED APPLICATIONS

Reference is made to the following commonly assigned, copending patent application, U.S. patent application Ser. No. 11/861,706, filed Sep. 26, 2007, entitled, "Single Component Developer." The disclosure of this patent application is hereby incorporated by reference in its entirety.

## BACKGROUND

Described herein are single component developers for use in forming and developing high gloss images in electrostaticographic, including xerographic, apparatuses. In embodiments, the toner is produced using emulsion aggregation processes. In embodiments, the toner is non-magnetic.

Emulsion aggregation toners can be used in electrophotography, including printing, copying, scanning, faxing, and the like, and including digital, image-on-image, and the like. The toner particles herein, in embodiments, can be made to have relatively uniform sizes, are nearly spherical in shape, and are environmentally friendly. U.S. patents describing emulsion aggregation toners include, for example, U.S. Pat. Nos. 5,370,963, 5,418,108, 5,290,654, 5,278,020, 5,308,734, 5,344,738, 5,403,693, 5,364,729, 5,346,797, 5,348,832, 5,405,728, 5,366,841, 5,496,676, 5,527,658, 5,585,215, 5,650,255, 5,650,256, 5,501,935, 5,723,253, 5,744,520, 5,763,133, 5,766,818, 5,747,215, 5,827,633, 5,853,944, 5,804,349, 5,840,462, 5,869,215, 6,803,166, 6,808,851, 6,824,942, 6,828,073, 6,830,860, 6,841,329, 6,849,371, 6,850,725, 6,890,696, 6,899,987, 6,916,586, 6,933,092, 6,936,396, 6,942,954, 6,984,480, 7,001,702, 7,029,817, 7,037,633, 7,041,420, 7,041,425, 7,049,042, 7,052,818, 7,097,954, 7,157,200, 7,160,661, 7,166,402, 7,179,575, 7,186,494, 7,208,253, and 7,217,484, each incorporated herein by reference in its entirety.

One main type of emulsion aggregation toner includes emulsion aggregation toners that include styrene acrylate resin. See, for example, U.S. Pat. No. 6,120,967, incorporated herein by reference in its entirety, as one example.

Emulsion aggregation techniques typically involve the formation of an emulsion latex of the resin particles, which particles have a small size of, for example, from about 5 to about 500 nanometers in diameter, by heating the resin, optionally with solvent if needed, in water, or by making a latex in water using an emulsion polymerization. A colorant dispersion, for example of a pigment dispersed in water, optionally also with additional resin, is separately formed. The colorant dispersion is added to the emulsion latex mixture, and an aggregating agent or complexing agent is then added to form aggregated toner particles. The aggregated toner particles are optionally heated to enable coalescence/fusing, thereby achieving aggregated, fused toner particles.

U.S. Pat. No. 5,462,828 describes a toner composition that includes a styrene/n-butyl acrylate copolymer resin having a number average molecular weight (Mn) of less than about 5,000, a weight average molecular weight of from about 10,000 to about 40,000, and a molecular weight distribution of greater than 6, that provides improved gloss and high fix properties at a low fusing temperature.

## SUMMARY

Disclosed in embodiments herein, is a toner for developing electrostatic images in a single component development sys-

## 2

tem, the toner comprising emulsion aggregation toner particles comprising a styrene acrylate polymer binder resin having a weight average molecular weight (Mw) of from about 50 to about 100 Kpse, and a number average molecular weight (Mn) of from about 10 to about 30 Kpse, a wax selected from the group consisting of polypropylene and polyethylene, and at least one colorant, wherein the toner particles have an onset glass transition temperature of from about 50° C. to about 60° C., and a circularity of from about 0.950 to about 0.990.

Embodiments further include a set of four toners for developing electrostatic images in a single component development system, wherein the set of four toners comprises a cyan toner, a magenta toner, a yellow toner and a black toner, and wherein each of the toners is a single component developer free of carrier and each of the cyan toner, magenta toner and yellow toners comprise emulsion aggregation toner particles comprising a styrene acrylate polymer binder having a weight average molecular weight (Mw) of from about 50 to about 100 Kpse and a number average molecular weight (Mn) of from about 10 to about 30, a wax selected from the group consisting of polyethylene and polypropylene, and at least one colorant, and further wherein the toner particles have an onset glass transition temperature of from about 50° C. to about 60° C., and a circularity of from about 0.950 to about 0.990.

Embodiments further include an emulsion aggregation toner comprising emulsion aggregation toner particles comprising a core and a shell, wherein the emulsion aggregation toner particles comprise a styrene acrylate polymer binder resin having a weight average molecular weight (Mw) of from about 50 to about 100 Kpse and a number average molecular weight (Mn) of from about 10 to about 30 Kpse, a wax selected from the group consisting of polypropylene and polyethylene, and at least one colorant, wherein the toner particles have an onset glass transition temperature of from about 50° C. to about 60° C., and a circularity of from about 0.950 to about 0.990, and wherein said core and shell both comprise the same styrene n-butyl acrylate polymer binder resin.

## DETAILED DESCRIPTION

in embodiments, the toner herein is robust and provides improved performance in single component development (SCD) systems. The toners herein, in embodiments, include a relatively high glass transition temperature and relatively high molecular weight latex resin, thereby providing improved anti-blocking and storage characteristics. The toners herein, in embodiments, include an additive package including silica and/or titania. Moreover, in embodiments, the toner herein has a near spherical shape, which, along with the additive package, provides for improved toner flow, which is desired for single component development. The toner herein, in embodiments, also demonstrates improved release from the fuser member, partially enabled by the well-dispersed internal wax. The wax component is also well encapsulated into the particles, in embodiments, producing low toner cohesion. In embodiments, the toner is non-magnetic toner.

For single component developers, i.e., developers that contain no carriers, it is desired for the toner particles to exhibit high transfer efficiency (including excellent flow properties and low cohesivity) and an ability to take on an appropriate triboelectric charge. The toners described herein, in embodiments, possess appropriate compositions and physical properties to be ideally suited for use in single component developer machines.

## Toner Resin

The toner particles described herein comprise a toner latex resin. In embodiments, the resin comprises a styrene acrylate polymer. Illustrative examples of specific styrene acrylate polymer resins for the binder include poly(styrene-alkyl acrylate), poly(styrene-alkyl methacrylate), poly(styrene-alkyl acrylate-acrylic acid), poly(styrene-alkyl methacrylate-acrylic acid), poly(styrene-alkyl acrylate-acrylonitrile-acrylic acid), poly(styrene-propyl acrylate), poly(styrene-butyl acrylate), poly(styrene-butyl acrylate-acrylic acid), poly(styrene-butyl acrylate-methacrylic acid), poly(styrene-butyl acrylate-acrylonitrile), poly(styrene-butyl acrylate-acrylonitrile-acrylic acid), poly(styrene-butyl acrylate-betacarboxyethylacrylate), and other similar styrene acrylate. In embodiments, resin comprises a styrene n-butyl acrylate copolymer.

In embodiments, the styrene acrylate copolymer resin as prepared into a toner particle has a glass transition temperature (Tg) of from about 50° C. to about 60° C., or from about 54° C. to about 57° C. The Tg can be measured using DSC. In addition, the weight average molecular weight (Mw) of the resin is from about 50 to about 100 kpse, or from about 55 to about 85 kpse, or from about 57 to about 80 kpse. In embodiments, the resin has a number average molecular weight (Mn) of from about 10 to about 30, or from about 12 to about 22 Kpse. The Mw and Mn can be measured using GPC. The resin comprises from about 30 to about 50 percent, or from about 41 to about 45 percent solids.

The monomers used in making the polymer binder are not limited, and may include any one or more of, for example, styrene, acrylates such as methacrylates, butylacrylates,  $\beta$ -carboxyethyl acrylate ( $\beta$ -CEA), ethylhexyl acrylate, octylacrylate, etc., butadiene, isoprene, acrylic acid, methacrylic acid, itaconic acid, acrylonitrile, etc., and the like. Known chain transfer agents can be used to control the molecular weight properties of the polymer. Examples of chain transfer agents include dodecanthiol, dodecylmercaptan, octanethiol, carbon tetrabromide, carbon tetrachloride, and the like, in various suitable amounts, for example of about 0.1 to about 10 percent by weight of monomer, or about 0.2 to about 5 percent by weight of monomer. Also, crosslinking agents such as decanedioildiacrylate or divinylbenzene may be included in the monomer system in order to obtain higher molecular weight polymers, for example in an effective amount of about 0.01 percent by weight to about 25 percent by weight, or from about 0.25 to about 5 percent by weight.

In an embodiment, the monomer components, with any of the aforementioned optional additives, are formed into a latex emulsion and then polymerized to form small-sized polymer particles, for example on the order of from about 100 nm to about 400 nm, or about 150 nm to about 300 nm, or from about 170 to about 250 nm.

The monomers and any other emulsion polymerization components may be polymerized into a latex emulsion with or without the use of suitable surfactants. Any other suitable method for forming the latex polymer particles from the monomers may be used.

In an embodiment, the toner particles have a core-shell structure. In this embodiment, the core comprises toner particle materials discussed above, including at least a binder, colorant, and wax. Once the core particle is formed and aggregated to a desired size, as will be discussed further below, a thin outer shell is then formed upon the core particle. The shell may comprise binder material (i.e., free of colorant, release agent, etc.), although other components may be included therein if desired.

The shell can comprise a latex resin that is the same or different from that of the core particle. In embodiments, the

core comprises a styrene acrylate resin and the shell comprises a styrene acrylate resin. In embodiments, both the core and the shell comprise a styrene n-butyl acrylate copolymer. The core latex may be added in an amount of from about 50 to about 80 percent, or from about 60 to about 75 percent by weight of total solids. The shell latex may be added to the toner aggregates in an amount of about 20 to about 50 percent, or from about 25 to about 40 percent by weight of the total binder materials.

10 In embodiments, the shell resin may have either the same, higher or a lower glass transition temperature (Tg) than the binder of the toner core particle. A higher Tg may be desired to limit penetration of the external additives and/or wax into the shell, while a lower Tg shell may be desired where greater penetration of the external additives and/or wax is desired. A higher Tg shell may also lend better shelf and storage stability to the toner. In embodiments, both the core and shell resins have a Tg of from about 50° C. to about 60° C., or from about 54° C. to about 57° C. as measured by DSC.

## 20 Colorants

Various known colorants, such as pigments, dyes, or mixtures thereof, can be present in the toner in an effective amount of, for example, from about 1 to about 10 percent by weight of toner, or from about 1 to about 5, or from about 1.25 to about 4 percent by weight, that can be selected include black, cyan, violet, magenta, orange, yellow, red, green, brown, blue or mixtures thereof.

Examples of a black pigment include carbon black, copper oxide, manganese dioxide, aniline black, activated carbon, non-magnetic ferrite and magnetite and the like, and wherein the magnetites, especially when present as the only colorant component, can be selected in an amount of up to about 70 weight percent of the toner. However, in embodiments, the toner is non-magnetic.

35 Specific examples of blue pigment include Prussian Blue, cobalt blue, Alkali Blue Lake, Victoria Blue Lake, Fast Sky Blue, Indanthrene Blue BC, Aniline Blue, Ultramarine Blue, Calco Oil Blue, Methylene Blue Chloride, Phthalocyanine Blue, Phthalocyanine Green and Malachite Green Oxalate or mixtures thereof. Specific illustrative examples of cyans that may be used as pigments include Pigment Blue 15:1, Pigment Blue 15:2, Pigment Blue 15:3 and Pigment Blue 15:4, copper 40 tetra(octadecyl sulfonamido)phthalocyanine, x-copper phthalocyanine pigment listed in the Color index as CI 74160, CI Pigment Blue, and Anthrathrene Blue, identified in the Color index as CI 69810, Special Blue X-2137, and the like.

45 Examples of a green pigment include Pigment Green 36, Pigment Green 7, chromium oxide, chromium green, Pigment Green, Malachite Green Lake and Final Yellow Green G.

50 Examples of a red or magenta pigment include red iron oxide, cadmium red, red lead oxide, mercury sulfide, Watchoung Red, Permanent Red 4R, Lithol Red, Naphthol Red, Brilliant Carmine 3B, Brilliant Carmine 6B, DuPont Oil Red, Pyrazolone Red, Rhodamine B Lake, Lake Red C, Rose Bengal, Eoxine Red and Alizarin Lake. Specific examples of magentas that may be selected include, for example, Pigment Red 49:1, Pigment Red 81, Pigment Red 122, Pigment Red 185, Pigment Red 238, Pigment Red 269, Pigment Red 57:1, 55 2,9-dimethyl-substituted quinacridone and anthraquinone dye identified in the Color Index as CI 60710, CI Dispersed Red 15, diazo dye identified in the Color index as CI 26050, CI Solvent Red 19, and the like.

60 Examples of a violet pigment include manganese violet, Fast Violet B and Methyl Violet Lake, Pigment Violet 19, Pigment Violet 23, Pigment Violet 27 and mixtures thereof.

Specific examples of an orange pigment include Pigment Orange 34, Pigment Orange 5, Pigment Orange 13, Pigment Orange 16, and the like. Other orange pigments include red chrome yellow, molybdenum orange, Permanent Orange GTR, Pyrazolone Orange, Vulkan Orange, Benzidine Orange G, Indanethrene Brilliant Orange RK and Indanethrene Brilliant Orange GK.

Specific examples of yellow pigments are Pigment Yellow 17, Pigment Yellow 74, Pigment Yellow 83, Pigment Yellow 93, Yellow 180, Yellow 185, and the like. Other illustrative examples of yellow pigment include chrome yellow, zinc yellow, yellow iron oxide, cadmium yellow, chrome yellow, Hansa Yellow, Hansa Yellow 10G, Hansa Brilliant Yellow, Benzidine Yellow G, Benzidine Yellow GR, Suren Yellow, Quinoline Yellow, Permanent Yellow NCG, diarylide yellow 3,3-dichlorobenzidene acetoacetanilides, a monoazo pigment identified in the Color Index as CI 12700, CI Solvent Yellow 16, a nitrophenyl amine sulfonamide identified in the Color Index as Foron Yellow SE/GLN, CI Dispersed Yellow 33 2,5-dimethoxy-4-sulfonanilide phenylazo-4'-chloro-2,5-dimethoxy acetoacetanilide, and Permanent Yellow FGL.

Examples of a white pigment include Pigment White 6, zinc white, titanium oxide, antimony white and zinc sulfide.

Colorants for use herein can include one or more pigments, one or more dyes, mixtures of pigment and dyes, mixtures of pigments, mixtures of dyes, and the like. The colorants are used solely or as a mixture.

Examples of a dye include various kinds of dyes, such as basic, acidic, dispersion and direct dyes, e.g., nigrosine, Methylene Blue, Rose Bengal, Quinoline Yellow and Ultramarine Blue.

A dispersion of colorant particles can be prepared by using a rotation shearing homogenizer, a media dispersing apparatus, such as a ball mill, a sand mill and an attritor, and a high pressure counter collision dispersing apparatus. The colorant can be dispersed in an aqueous system with a homogenizer by using a surfactant having polarity.

The colorant may be selected from the standpoint of hue angle, chroma saturation, brightness, weather resistance, OHP transparency and dispersibility in the toner. In the case where the colorant particles in the toner have a median diameter of from 100 to 330 nm, the OHP transparency and the coloration property can be assured. The median diameter of the colorant particles can be measured, for example, by a laser diffraction particle size measuring apparatus (MicroTrac UPA 150, produced by MicroTrac Inc.).

In the case where the toner is obtained in an aqueous system, it is necessary to attend to the aqueous phase migration property of the magnetic material, and in embodiments, the surface of the magnetic material is modified in advance, for example, subjected to a hydrophobic treatment.

#### Wax

In addition to the latex polymer binder and the colorant, the toners may also contain a release agent, in embodiments, a wax dispersion. The release agent is added to the toner formulation in order to aid toner offset resistance, e.g., toner release from the fuser member, particularly in low oil or oil-less fuser designs. Specific examples of suitable release agents include a polyolefin, such as polyethylene, polypropylene and polybutene, a silicone exhibiting a softening point upon heating, an aliphatic amide, such as oleic acid amide, erucic acid amide, ricinoleic acid amide and stearic acid amide, vegetable wax, such as carnauba wax, rice wax, candelilla wax, wood wax and jojoba oil, animal wax, such as bees wax, mineral or petroleum wax, such as montan wax, ozokerite, ceresin, paraffin wax, microcrystalline wax and

Fischer-Tropsch wax, and modified products thereof. In embodiments, a polyethylene wax such as POLYWAX® 725 can be used.

The release agent may be dispersed in water along with an ionic surfactant or a polymer electrolyte, such as a polymer acid and a polymer base, and it is heated to a temperature higher than the melting point thereof and is simultaneously dispersed with a homogenizer or a pressure discharge disperser (Gaulin Homogenizer) capable of applying a large 10 shearing force, so as to form a dispersion of particles having a median diameter of 1  $\mu\text{m}$  or less.

The release agent can be added in an amount of from about 5 to about 15 percent by weight, or from about 8 to about 12 percent by weight, or about 9 percent to about 10 percent, 15 based on the total weight of the solid content constituting the toner.

The particle diameter of the resulting release agent particle dispersion can be measured, for example, by a laser diffraction particle size measuring apparatus (Microtrac UPA 150 20 manufactured by MicroTrac Inc.). The release agent, in embodiments, has a particle size of less than about 1.0 micron. The resin fine particles, the colorant fine particles, and the release agent particles can be aggregated, and then the resin fine particle dispersion is added to attach the resin fine particles on the surface of the aggregated particles from the standpoint of assurance of charging property and durability.

#### Additives

The toner may also include additional known positive or negative charge additives in effective suitable amounts of 30 from about 0.1 to about 5 weight percent of the toner, or from about 0.1 to about 3 percent of the toner. Examples include titania, silica, cerium, tin oxide, aluminum oxide, and the like. Commercially available examples include MT-3103 Titania, R805 silica, and the like. In embodiments, silica is applied to 35 the toner surface for toner flow, tribe enhancement, improved development and transfer stability and higher toner blocking temperature. In embodiments,  $\text{TiO}_2$  is applied for improved relative humidity (RH) stability, tribe control and improved development and transfer stability. The external surface additives can be used with or without a coating. In addition, more than one of the same type of additive can be added, for example, two different silicas and/or two different titanias, and the like.

In embodiments, silica can have a particle size of from 45 about 5 to about 15 nm, or from about 8 to about 12 nm. The additives can be treated/coated with HMDS (hexamethyldisilazane) and/or a PDMS (polydimethylsiloxanes). The inorganic additive particles of this size range may exhibit a BET (Brunauer, Emmett and Teller) surface area of from about 100 to about 300  $\text{m}^2/\text{g}$ , or from about 125 to about 250  $\text{m}^2/\text{g}$ , although the values may be outside of this range as needed. Titania (titanium oxide) can have a size of from about 5 nm to about 130 nm, or from about 10 to about 30 nm. The titania particles can exhibit a BET surface area of from about 20 to 55 about 120  $\text{m}^2/\text{g}$ , or from about 30 to about 80  $\text{m}^2/\text{g}$ , although the values may be outside of this range as needed. The additive package may further include a second silica having a size larger than the first silica and having a size of from about 20 nm to about 150 nm, and optionally can be treated and/or coated with HMDS and/or PDMS. The larger size silica can acts as a spacer material. The larger size silica may be omitted, and no spacer material used, or an alternative spacer material used in its place, without restriction.

#### Surfactants

One or more surfactants may be used in the emulsion aggregation process. Suitable surfactants may include anionic, cationic and nonionic surfactants.

Anionic surfactants include sodium dodecylsulfate (SDS), sodium dodecyl benzene sulfonate, sodium dodecyl naphthalene sulfate, dialkyl benzenealkyl sulfates and sulfonates, and abitic acid. An example of suitable anionic surfactants is a branched sodium dodecyl benzene sulfonate.

Examples of cationic surfactants include dialkyl benzene alkyl ammonium chloride, lauryl trimethyl ammonium chloride, alkylbenzyl methyl ammonium chloride, alkyl benzyl dimethyl ammonium bromide, benzalkonium chloride, cetyl pyridinium bromide, C<sub>12</sub>, C<sub>15</sub>, C<sub>17</sub> trimethyl ammonium bromides, halide salts of quaternized polyoxyethylalkylamines, dodecyl benzyl triethyl ammonium chloride, benzalkonium chlorides, and the like. An example of a cationic surfactant is benzyl dimethyl alkonium chloride.

Examples of nonionic surfactants include polyvinyl alcohol, polyacrylic acid, methalose, methyl cellulose, ethyl cellulose, propyl cellulose, hydroxy ethyl cellulose, carboxy methyl cellulose, polyoxyethylene cetyl ether, polyoxyethylene lauryl ether, polyoxyethylene octyl ether, polyoxyethylene octylphenyl ether, polyoxyethylene oleyl ether, polyoxyethylene sorbitan monolaurate, polyoxyethylene stearyl ether, polyoxyethylene nonylphenyl ether, and dialkylphenoxy poly(ethyleneoxy)ethanol. An example of a nonionic surfactant is alkyl phenol ethoxylate.

#### Emulsion Aggregation

Any suitable emulsion aggregation (EA) procedure may be used in forming the emulsion aggregation toner particles without restriction. These procedures typically include the basic process steps of at least aggregating a latex emulsion containing binder, one or more colorants, optionally one or more surfactants, optionally a wax emulsion, optionally a coagulant and one or more additional optional additives to form aggregates, optionally forming a shell on the aggregated core particles as discussed above, subsequently optionally coalescing or fusing the aggregates, and then recovering, optionally washing and optionally drying the obtained emulsion aggregation toner particles.

An example emulsion aggregation coalescing process includes forming a mixture of latex binder, colorant dispersion, optional wax emulsion, optional coagulant and deionized water in a vessel. In known methods, the mixture is then sheared using a homogenizer until homogenized and then transferred to a reactor where the homogenized mixture is heated to a temperature of, for example, at least about 50° C., or about 60° C. to about 70° C. and held at such temperature for a period of time to permit aggregation of toner particles to a desired size. However, in embodiments, the mixture is mixed at a temperature above the T<sub>g</sub> of the resin, or from about 60 to about 70, or from about 62 to about 70° C., and held at such temperature for a period of time to permit aggregation of toner particles to a desired size. In this regard, aggregation refers to the melding together of the latex, pigment, wax and other particles to form larger size agglomerates. Once a desired core particle size is reached, additional latex binder may then be added to form a shell upon the aggregated core particles. In embodiments, the outer shell can be added until the appropriate particle size is reached, such as from about 5 to about 8, or from about 6 to about 8, or from about 7 to about 7.5  $\mu\text{m}$ . Once the desired size of aggregated toner particles is achieved, aggregation is then halted, for example by adjusting the pH of the mixture in order to inhibit further toner aggregation, such as by adding ammonium hydroxide. The toner particles are then coalesced at a temperature of at least about 80° C., or from about 90° C. to about 100° C., and the pH adjusted in order to enable the particles to coalesce and spherodize (become more spherical and smooth). The desired and shape and morphology are obtained

and they depend on the amount of wax protrusions desired on the surface of the particle and the shape of the particle. The mixture is then cooled to a desired temperature, at which point the aggregated and coalesced toner particles are recovered and optionally washed and dried or they are wet sieved washed by filtration and then dried.

The toner particles are blended with external additives following formation. Any suitable surface additives may be used.

- 10 In embodiments, the toner particles are made to have a volume mean diameter of from about 5 to about 8, or from about 6 to about 8, or from about 7 to about 7.5  $\mu\text{m}$ . The toners herein can have an average circularity of about 0.950 to about 0.990, or from about 0.960 to about 0.980, and a volume and 15 number geometric standard deviation (GSD<sub>v and n</sub>) of from about 1.10 to about 1.30, or from about 1.15 to about 1.25, or from about 1.20 to about 1.23. The average particle size refers to a volume average size that may be determined using any suitable device, for example a conventional Coulter counter. 20 The circularity may be determined using any suitable method, for example the known Malvern Sysmex Flow Particle Integration Analysis method. The circularity is a measure of the particles closeness to perfectly spherical. A circularity of 1.0 identifies a particle having the shape of a perfect circular 25 sphere. The GSD refers to the upper geometric standard deviation (GSD) by volume (coarse level) for (D84/D50) and can be from about 1.10 to about 1.30, or from about 1.15 to about 1.25, or from about 1.20 to about 1.23. The geometric standard deviation (GSD) by number (fines level) for (D50/D16) can be from about 1.10 to about 1.30, or from about 1.15 to about 1.25, or from about 1.23 to about 1.25. The particle diameters at which a cumulative percentage of 50% of the total toner particles are attained are defined as volume D50, 30 and the particle diameters at which a cumulative percentage of 84% are attained are defined as volume D84. These aforementioned volume average particle size distribution indexes GSD<sub>v</sub> can be expressed by using D50 and D84 in cumulative distribution, wherein the volume average particle size distribution index GSD<sub>v</sub> is expressed as (volume D84/volume D50). These aforementioned number average particle size distribution indexes GSD<sub>n</sub> can be expressed by using D50 and D16 in cumulative distribution, wherein the number average particle size distribution index GSD<sub>n</sub> is expressed as (number D50/number D16). The closer to 1.0 that the GSD 35 value is, the less size dispersion there is among the particles. The aforementioned GSD value for the toner particles indicates that the toner particles are made to have a narrow particle size distribution.

The toners herein provide a shaper factor or circularity of 40 from about 0.950 to about 0.990, or from about 0.960 to about 0.980. In addition, the toners herein have an onset T<sub>g</sub> of from about 50 to about 60, or from about 53 to about 58, or about 55° C.

The toner particles described herein can be used as single 45 component developer (SCD) formulations that are free of carrier particles.

The aforementioned toner particles as a single component developer composition in SCD deliver a very high transfer efficiency.

- 60 Typically in SCD, the charge on the toner is what controls the development process. The donor roll materials are selected to generate a charge of the right polarity on the toner when the toner is brought in contact with the roll. The toner layer formed on the donor roll by electrostatic forces is passed 65 through a charging zone, specifically in this application a charging roller, before entering the development zone. Light pressure in the development nip produces a toner layer of the

desired thickness on the roll as it enters the development zone. This charging typically will be for only a few seconds, minimizing the charge on the toner. An additional bias is then applied to the toner, allowing for further development and movement of the controlled portion of toner to the photoreceptor. If the low charge toner is present in sufficient amounts, background and other defects become apparent on the image. The image is then transferred from the photoreceptor to an image receiving substrate, which transfer may be direct or indirect via an intermediate transfer member, and then the image is fused to the image receiving substrate, for example by application of heat and/or pressure, for example with a heated fuser roll.

The toner and developer will now be further described via the following examples.

The following Examples further define and describe embodiments herein. Unless otherwise indicated, all parts and percentages are by weight.

## EXAMPLES

### Example 1

#### Synthesis of Latex(Toner Resin)

A latex was prepared by semicontinuous emulsion polymerization of styrene/butyl acrylate/ $\beta$ -carboxyethylacrylate, 75/25/3 parts (by weight), and using a diphenyloxide disulfonate surfactant as follows. An 8 liter jacketed glass reactor was fitted with two stainless steel 450 pitch semi-axial flow impellers, thermal couple temperature probe, water cooled condenser with nitrogen outlet, a nitrogen inlet, internal cooling capabilities, and hot water circulating bath. After reaching a jacket temperature of 820° C. +/− 1.00° C. and continuous nitrogen purge, the reactor was charged with 1779.98 grams of distilled water and 2.89 grams of Dowfax 2A1™. The stirrer was then set at 200 RPM and maintained at this speed for 2 hours. The reactor contents were controlled at 750° C. +/− 0.40° C. by the internal cooling system. A monomer emulsion was prepared by combining 1458.7 grams of styrene, 486.2 grams of n-butyl acrylate, 58.4 grams of  $\beta$ -carboxyethylacrylate, and 9.7 grams of dodecylmercaptan, with an aqueous solution of 38.4 grams of DOWFAX 2A1™, and 921.5 grams of distilled water. The mixture was then subjected to a series of on/off high shear mixing to form a stable emulsion.

From the prepared stable emulsion, about 59.5 grams was transferred into the reactor and stirred for approximately 10 minutes to maintain a stable emulsion, and to allow the reactor contents to equilibrate at 750° C. An initiator solution prepared from 38.89 grams of ammonium persulfate in 134.7 grams of distilled water was then added over a period of 20 minutes by pump to the reactor contents. This was immediately followed by flushing the pump with about 9.5 grams of distilled water into the reactor. Stirring continued for an additional 20 minutes to allow seed particle formation. The remaining approximate 2913.5 grams of monomer emulsion were then fed continuously into the reactor over a period of about 193 minutes, followed immediately by an additional distilled water flush of about 45 grams. After monomer emulsion addition was completed, the reaction was allowed to post react for about 180 minutes at 750 C. At this time the reactor and contents was cooled to room temperature and the latex removed.

The resulting latex polymer possessed a Mw of about 51,500, a Mn of about 13,600, as determined by GPC, and a onset Tg of approximately 56.80 C by DSC. The latex resin

possessed a volume average diameter of 231 nanometers measured on a Microtrac light scattering instrument.

### Example 2

#### Cyan Toner Preparation

A 50 kpse Mw latex, P725 wax, cyan pigment, and Polyaluminum chloride were charged into the reactor. The mixture was homogenized for 50 minutes until thoroughly mixed. The aggregation temperature was set to 57° C. and the rpm was set to 280. The measured aggregate size before shell addition was 6.49  $\mu$ m. The jacket temperature was then set to 570° C. at shell addition. The aggregation time before the shell latex addition was 74 minutes. The latex shell was then added within 14 minutes. The aggregation time after latex shell addition was 38 minutes and the particle frozen with base (1M NaOH) at 7.41  $\mu$ m, pH 4.7. The coalescence pH was done with 0.3M HNO<sub>3</sub> at pH 3.8. The circularity of the particle at time zero, and 960° C. was 0.937. The final circularity was read at 120 minutes and found to be 0.980. The batch was then cooled to 630° C. at 0.70° C./min, the pH increased to 10 and the batch was treated for 20 minutes before washing. The final particle results were: D50=7.08  $\mu$ m; GSDv=1.21; GSDn=1.23; Vol Ratio 84/50=1.12; and Nmb Ratio 50/16=1.25.

These particles were blended with 0.8% RY50 SiO<sub>2</sub> and 0.8% R805 SiO<sub>2</sub> and 0.8% RY50 SiO<sub>2</sub> and 1.0% R805 SiO<sub>2</sub> and 0.1, 0.2 or 0.30 MT3103 TiO<sub>2</sub> to produce functional toner.

### Example 3

#### Yellow Toner Preparation

A 50 kpse Mw latex, P725 wax, yellow pigment, and Polyaluminum chloride was charged into the reactor. The mixture was homogenized for 50 minutes until thoroughly mixed. The aggregation temperature was set to 57° C. and the rpm was set to 320. The measured aggregate size before shell addition was 6.19  $\mu$ m. The jacket temperature was then set to 570° C. at shell addition. The aggregation time before the shell latex addition was 96 minutes. The latex shell was then added within 15 minutes. The aggregation time after latex shell addition was 83 minutes and the particle frozen with base (1M NaOH) at 7.50  $\mu$ m, pH 4.7. The coalescence pH was met by using 0.3M HNO<sub>3</sub> at pH 3.8. The circularity of the particle at time zero, and 960° C. was 0.927. The final circularity was read at 270 minutes and found to be 0.976. The batch was then cooled to 630° C. using 0.70° C./min, the pH increased to 10 and the batch was treated for 20 minutes before washing. The final particle results were: D50=7.15  $\mu$ m; GSDv=1.20; GSDn=1.23; Vol Ratio 84/50=1.19; and Nmb Ratio 50/16=1.24.

These particles were blended with 0.8% RY50 SiO<sub>2</sub> and 1.0% R805 SiO<sub>2</sub> and 0.1, 0.2 or 0.30 MT3103 TiO<sub>2</sub> to produce functional toner.

### Example 4

#### Magenta Toner Preparation

Preparation of Ea SCD Magenta Toner by A/C Process was Initiated using 50 kpse Mw latex, P725 wax, magenta pigments, and Polyaluminum chloride charged into a reactor. The mixture was homogenized for 50 minutes until thoroughly mixed. The aggregation temperature was set to 57° C. and the rpm was set to 350. The measured aggregate size

## 11

before shell addition was 6.47  $\mu\text{m}$ . The jacket temperature was then set to 570° C. at shell addition. The aggregation time before the shell latex addition was 65 minutes. The latex shell was then added within 15 minutes. The aggregation time after latex shell addition was 65 minutes and the particle frozen with base (1M NaOH) at 7.49  $\mu\text{m}$ , pH 4.7. The coalescence pH was done with 0.3M HNO<sub>3</sub> at pH 3.8. The circularity of the particle at time zero, and 960° C. was 0.930. The final circularity was read at 240 minutes and found to be 0.978. The batch was then cooled to 630° C. at 0.70° C./min, the pH increased to 10 and the batch was treated for 20 minutes before washing. The final particle results were: D50=7.54  $\mu\text{m}$ ; GSDv=1.21; GSDn=1.24; Vol Ratio 84/50=1.20; and Nmb Ratio 50/16=1.26.

These particles had been blended with 1.25% R805 SiO<sub>2</sub> and 0.1, 0.2 or 0.30 MT3103 TiO<sub>2</sub> to produce functional toner.

## Example 5

## Black Toner Preparation

Preparation of Ea SCD Black Toner Particles by A/C Process Includes 50 kpse Mw latex, P725 wax, black pigment, and Polyaluminum chloride being charged into a reactor. The mixture was homogenized for 50 minutes until thoroughly mixed. The aggregation temperature was set to 57° C. and the rpm was set to 300. The measured aggregate size before shell addition was 6.14  $\mu\text{m}$ . The jacket temperature was then set to 570° C. at shell addition. The aggregation time before the shell latex addition was 72 minutes. The latex shell was then added within 15 minutes. The aggregation time after latex shell addition was 25 minutes and the particle was frozen with base (1M NaOH) at 7.44  $\mu\text{m}$ , pH 4.7. The coalescence pH was done with 0.3M HNO<sub>3</sub> at pH 3.8. The circularity of the particle at time zero, and 960° C. was 0.939. The final circularity was read at 120 minutes and found to be 0.978. The batch was then cooled to 630 C at 0.70° C./min, the pH increased to 10 and treated for 20 minutes before washing. The final particle results were: D50=7.09  $\mu\text{m}$ ; GSDv=1.19; GSDn=1.23; Vol Ratio 84/50=1.18; Nm Ratio 50/16=1.25.

These particles had been blended with 1.25% R805 SiO<sub>2</sub> and 0.1, 0.2 or 0.30 MT3103 TiO<sub>2</sub> to produce functional toner.

It will be appreciated that various of the above-disclosed and other features and functions, or alternatives thereof, may be desirably combined into many other different systems or applications. Also, various presently unforeseen or unanticipated alternatives, modifications, variations or improvements therein may be subsequently made by those skilled in the art, and are also intended to be encompassed by the following claims.

The claims, as originally presented and as they may be amended, encompass variations, alternatives, modifications, improvements, equivalents, and substantial equivalents of the embodiments and teachings disclosed herein, including those that are presently unforeseen or unappreciated, and that, for example, may arise from applicants/patentees and others.

What is claimed is:

1. A toner for developing electrostatic images in a single component development system, said toner comprising emulsion aggregation toner particles comprising a styrene acrylate

## 12

polymer binder resin having a weight average molecular weight (Mw) of from about 50,000 to about 100,000 Daltons, and a number average molecular weight (Mn) of from about 10,000 to about 30,000 Daltons, a wax selected from the group consisting of polypropylene and polyethylene, and at least one colorant, wherein the toner particles have an onset glass transition temperature of from about 50° C. to about 60° C., and a circularity of from about 0.950 to about 0.990.

2. A toner as in claim 1, wherein both the toner particles and the shell comprise a same styrene acrylate polymer.

3. A toner as in claim 1, wherein said styrene acrylate polymer is a styrene n-butyl acrylate copolymer.

4. A toner as in claim 1, wherein said resin has a weight average molecular weight (Mw) of from about 55,000 to about 85,000 Daltons, and a number average molecular weight (Mn) of from about 12,000 to about 22,000 Daltons.

5. A toner as in claim 1, wherein said resin comprises from about 30 to about 50 percent solids.

6. A toner as in claim 1, wherein said toner has a Tg of from about 54 to about 57° C.

7. A toner as in claim 1, wherein the toner particles have circularity of from about 0.960 to about 0.980.

8. A toner as in claim 1, wherein said toner has a volume mean diameter of from about 5 to about 8  $\mu\text{m}$ .

9. A toner as in claim 1, wherein said toner has an upper geometric standard deviation (D84/D50) of from about 1.10 to about 1.30.

10. A toner as in claim 1, wherein said toner has a lower geometric standard deviation (D50/D16) of from about 1.10 to about 1.30.

11. A set of four toners for developing electrostatic images in a single component development system, wherein said set of four toners comprises a cyan toner, a magenta toner, a yellow toner and a black toner, and wherein each of the toners is a single component developer free of carrier and each of the cyan toner, magenta toner and yellow toners comprise emulsion aggregation toner particles comprising a styrene acrylate polymer binder having a weight average molecular weight (Mw) of from about 50,000 to about 100,000 Daltons and a number average molecular weight (Mn) of from about 10,000 to about 30,000 Daltons, a wax selected from the group consisting of polyethylene and polypropylene, and at least one colorant, and further wherein the toner particles have an onset glass transition temperature of from about 50° C. to about 60° C., and a circularity of from about 0.950 to about 0.990.

12. An emulsion aggregation toner comprising emulsion aggregation toner particles comprising a core and a shell, wherein said emulsion aggregation toner particles comprise a styrene acrylate polymer binder resin having a weight average molecular weight (Mw) of from about 50,000 to about 100,000 Daltons and a number average molecular weight (Mn) of from about 10,000 to about 30,000 Daltons, a wax selected from the group consisting of polypropylene and polyethylene, and at least one colorant, wherein the toner particles have an onset glass transition temperature of from about 50° C. to about 60° C., and a circularity of from about 0.950 to about 0.990, and wherein said core and shell both comprise the same styrene n-butyl acrylate polymer binder resin.

\* \* \* \* \*